

Patented Dec. 29, 1925.

## UNITED STATES PATENT OFFICE.

JOHANNES HELL, OF ESSLINGEN, GERMANY.

## TANNING OF SKINS AND HIDES.

No Drawing.

Application filed August 29, 1921. Serial No. 496,597.

*To all whom it may concern:*

Be it known that I, JOHANNES HELL, a citizen of the Republic of Germany, and resident of Esslingen, Wurttemberg, Germany, have invented certain new and useful Improvements in or Relating to the Tanning of Skins and Hides, of which the following is a specification.

The present invention relates to an improved process of tanning hides and skins under which I also include those in a partially tanned condition.

According to the present invention hides or skins are tanned by means of soluble magnesium salts (such as the sulphate or the chloride) and soluble carbonic acid salts (such as the carbonate or bicarbonate of sodium) in the presence of water. The magnesium salts and the carbonic acid salts of other bases may in this process be employed either simultaneously or successively. For instance in the working of this process, the wet hides or skins may be introduced into a drum, and a mixture of dry magnesium sulphate and sodium bicarbonate is then added. The moisture in the hides or skins as usually prepared, will in certain cases be found sufficient to dissolve the salts and render them active; or the hides and skins may be drummed in a solution of magnesium sulphate, and sodium carbonate or sodium bicarbonate added thereto subsequently; or the hides and skins may first be drummed in a solution of carbonate or bicarbonate of sodium and the magnesium sulphate added afterwards.

My improved process is a true tanning process as distinguished from a liming process.

I am not prepared to state with any degree of certainty what chemical changes—leading to the formation of leather—occur between the soluble magnesium salts, the soluble carbonic acid salts of other bases and the hide substances, but the latter undoubtedly plays an important part. In all probability the tannage which occurs, results from a precipitation in and upon the hides or skins, of one or more insoluble magnesium compounds which are either salts of carbonic acid or contain such salts. In order to secure the best results it is necessary to incorporate a certain minimum quantity of the magnesium carbonate in the skin, and preferably in concentrated solution. It is also important for the securing

of the best results that the product should not be washed immediately after removal from the bath, as apparently the reaction continues for several hours, or the reaction products do not become fixed at once. Whatever may be the exact changes, the fact remains that the hides or skins undergo a change and leather is produced which leather remains permanent and cannot be re-converted into the condition of a skin, even though the tanned hides or skins be washed, for example, with water a few hours after the treatment.

My tanning process may be performed in a very short time compared to that required for most tanning processes, and the materials used are inexpensive and easily obtained. The leather obtained may be sold and used without further tanning operation, or the character of the leathers obtained with this improved process may be greatly varied or modified by the application in conjunction therewith or thereafter of tanning processes or substances already known. For example, valuable results may be attained if the hides or skins in addition to being treated by the above process are also subjected to the action of other tanning agents such as cellulose extract, formaldehyde, metallic or other tanning salts or other tanning substances.

These substances may be used upon the hides or skins by themselves or in admixture one with the other or after one another at any time in proper conjunction with the "magnesium tannage" above referred to. They may also be used during or after the currying of the leather.

In certain cases, for instance, where vegetable tanning methods are used, the magnesium tanned leather must be freed from excess of alkali, but in other cases the tanning agents may be added during the process of the magnesium tannage.

The following examples are only a few actual methods for carrying the invention into effect.

1. 100 kg. of unhaired hide are worked for 4 to 6 hours, or longer if necessary, with a concentrated solution containing 21-22 kg. of magnesium sulphate and 7 kg. of sodium bicarbonate or 9 kg. sodium carbonate, in a drum. The solutions may be prepared either before or after the hides are introduced into the drum or the hides may first of all be brought into the mag-

nesium sulphate solution, and the carbonate or bicarbonate solution added subsequently, or vice versa. The leather thus obtained may be rinsed and then oiled. The 5 resultant product is soft, tough, and of enlarged area.

2. The hide treated according to Example 1 is pressed out or exposed to the air, then 10 coated or brushed over with cellulose extract (purified cellulose sulphite liquor) and thereafter rolled and greased. The leather thus obtained possesses considerable body and retains the form which it is given during staking or currying and does not shrink 15 any further. Similar advantages may be obtained, if an appropriate quantity of cellulose extract is added to the tanning mixture.

3. By treatment with formalin, for example 20 by the addition of about 1 litre of 40% formaldehyde to the tanning solution described in Example 1, leather with a property of resisting heat and alkali is obtained.

When subjected to the action of heat, 25 which destroys vegetable tanned leather, the leather prepared according to this example remains flat after cooling, as well as pliant, tough or stable in grain. Even if such leather has been dried without greasing, 30 it will not crack when subjected to strong bending.

The currying of such leathers may be carried out with or without cellulose extract. The greased leather is particularly 35 tough and strong in the grain; it can readily be curried to any grain, thereby dispensing with the otherwise usual softening operations.

4. By steeping the leather obtained in accordance with Example 1, in dilute formaldehyde solution, or coating it with such 40 solution, or with fat, grease or the like to which formaldehyde has been added, the leather attains, amongst others, the property valuable for the production of imitation grain leather, so that the graining produced, for example, by plating or embossing, 45 is extremely durable. After drying, the graining thus produced cannot be removed permanently even by rolling or pressing the leather with hot plates.

5. If to the tanning mixture described in Example 1 an aqueous solution of 5 kg. of chrome alum is added, or if the leather obtained 50 in accordance with Example 1 is treated afterwards with a chrome tanning liquor, a leather is obtained which in addition to the good qualities obtained through the "magnesium tannage" has also the characteristics of chrome tanning. In the place of chromium salts the partly or completely prepared leather can also be treated with other salt solutions, such as salts of iron, zinc or barium.

6. By suitable joint application of com-

paratively small quantities of vegetable tanning materials, the leathers obtained by the "magnesium tannage" can be given the properties of those tanned with vegetable substances. For example, by the addition of 1 litre of oak extract of 20 to 25° Bé. to the 70 tanning solutions of Examples 1 or 3, leather is obtained which appears internally and externally like leather tanned with vegetable material. By any re-tanning process 75 leather of any usual leather-shade may be obtained which according to the material and method of re-tanning used, will produce either firm or soft leather and the substance of the resulting leather may be varied.

7. By alternately treating the skins in different baths, particular products can be attained. For example, a full bodied leather, firm and unbreakable on its grained side can be obtained, without even greasing, if the hide tanned in accordance with Example 3, is placed for some hours in milk of lime and then further treated as in Example 1.

8. Leather which has been obtained according to the treatment given in the above examples, with the exception of the treatment with formaldehyde and chrome salts, is treated in the finished state with formaldehyde, for example by coating with formaldehyde solution thereon. By this means previous artificially obtained unevenness of the leather is made unremovable.

As the fleshy side of the hides during 100 tanning according to this invention becomes finely grained and smooth, the process is particularly suitable for the tanning of split skins. Their finished appearance is better than with other tanning processes. 105 Artificially obtained grainings cannot be removed after the completion of the tanning.

In tanning hides in the hair, the invention gives the advantage that when for example formaldehyde is used, such hides are 110 quickly penetrated by the mixture.

The leather produced by the "magnesium tannage" supplemented by another tanning process may have all the qualities of a leather produced by the previously known 115 process alone, but there is great economy in time required, and in the quantity of the tanning material required for the supplemental process.

Having thus described my invention, 120 what I claim as new and desire to secure by Letters Patent is:—

1. The process of tanning skins or hides, consisting in incorporating carbonic acid salts of magnesium within the skins or 125 hides, and in sufficient quantity to effect tanning action.

2. The process of tanning skins or hides, consisting in treating them with materials capable of forming magnesium carbonates 130

within or in the presence of the skin or hide.

3. The process of tanning skins or hides, consisting in treating the skins or hides with soluble magnesium salts and soluble carbonic acid salts of another base in the presence of water.

4. The process of tanning skins or hides, consisting in effecting a reaction between a soluble magnesium salt and a soluble carbonic acid salt to form an insoluble compound in the presence of the hide or skin to be tanned.

5. The process of tanning hides or skins which includes the drumming of the moist hide or skin in the presence of a magnesium salt and a carbonic acid salt of another base, such salts being soluble in water and in sufficient quantity to effect tanning action.

6. The process of tanning hides or skins consisting in treating the hides or skins with substances capable of forming insoluble compounds of magnesium in the presence of the hides or skins, whereby such insoluble compounds are incorporated in the body of the skin in an amount sufficient to produce tanning action.

7. The process of tanning hides or skins consisting in treating the hides or skins with substances which react in the body of the skin to produce carbonates of magnesium

in a sufficient quantity to produce the tanning action.

8. The process of tanning a hide or skin, consisting in treating the hide or skin with a soluble magnesium salt and a soluble carbonic acid salt of another base in the presence of water, and varying the character of the leather so produced by further tanning by another process.

9. The process of tanning a hide or skin consisting in treating the hide or skin with materials capable of forming magnesium carbonates within or in the presence of the hide, and with formaldehyde.

10. As an article of manufacture leather produced by the interaction of a soluble carbonic acid salt and a soluble magnesium salt in the presence of the hide or skin, and having a product of such action incorporated therein.

11. In the manufacture of leather from hides or skins, the step of preparing the hide or skin for a final tanning action, which preparatory step includes the treating of the hide or skin with substances reacting to form a substantially insoluble magnesium salt within the structure of the hide or skin.

In testimony whereof I have signed my name to this specification.

JOHANNES HELL.